# EUROPEAN PATENT SPECIFICATION

(11) **EP 3 159 424 B1**
(45) Date of publication and mention of the grant of the patent: **24.04.2019**
(21) Application number: 14895253.4
(22) Date of filing: 27.06.2014
(51) Int. Cl.: C22C 38/38, C22C 38/22, C22C 38/28, C22C 38/24, C21C 1/02, C21C 5/30, C21C 7/10, C21C 7/068, C21C 7/06, C21D 8/08, B22D 11/00, C21D 8/06, C21D 9/52, C21C 5/28, C22C 38/00, C22C 38/02, C22C 38/04, C21C 7/064

(54) **REBAR AND PREPARATION METHOD THEREOF**
BEWEHRUNGSSTAB UND HERSTELLUNGSVERFAHREN DAFÜR
BARRE D'ARMATURE ET SON PROCÉDÉ DE PRÉPARATION

(30) Priority: 18.06.2014 CN 201410273604
(43) Date of publication of application: 26.04.2017
(73) Proprietor: INSTITUTE OF RESEARCH OF IRON AND STEEL, JIANGSU PROVINCE/SHA-STEEL, CO. LTD, Suzhou, Jiangsu 215625 (CN)
(72) Inventor: ZHANG, Jianchun, Suzhou Jiangsu 215625 (CN); MA, Han, Suzhou Jiangsu 215625 (CN); HUANG, Wenke, Suzhou Jiangsu 215625 (CN); LI, Yang, Suzhou Jiangsu 215625 (CN); ZUO, Longfei, Suzhou Jiangsu 215625 (CN)
(74) Representative: Groth & Co. KB
(86) International application number: PCT/CN2014/080994
(87) International publication number: WO 2015/192391

(56) References cited:
- CN-A- 101 838 772
- CN-A- 103 556 058
- JP-A- 2001 342 548
- JP-A- 2001 342 548
- JP-A- 2002 285 298
- JP-A- 2002 285 298
- JP-A- 2004 143 496
- JP-A- 2013 166 992

## Description

### Technical Field

The present invention relates to a steel rebar and a production method thereof, which pertains to the field of alloy steel.

### Background of the Invention

Along with consciousness enhancing of ocean strategy of various countries and development of modern ocean science and technology, constructions of infrastructure such as huge cross-river or cross-sea bridges, seaport wharfs, and offshore buildings are entering into a peak season. Meanwhile, the durability problem of steel rebar used as a main structural material becomes increasingly prominent. The ocean environment is a relatively harsh corrosion environment in the nature, with its special conditions of high temperature, high humidity, and high salinity easily causing corrosion of steel. Severe corrosion usually occurs in the reinforced concrete structures along the coast of China after 10-15 years on service, which results in damage to the structures, rendering the structures unable to meet their designed service life of 50 years.

There are two major ways to increase the corrosion resistance performance of steel rebar in a concrete structure: the first way is applying organic or inorganic coatings onto carbon steel rebar, while the second way is alloying or various processing techniques to obtain steel rebar materials with excellent corrosion resistance performance. Among coated corrosion resistant steel rebar products, epoxy coated steel rebar is researched earliest and used most widely, however, epoxy coated steel rebar has essential disadvantages reflected as: the coating has high brittleness, and is easily damaged and shed off during transporting and processing; defects in the coating might cause concentrated corrosion which leads to severe local corrosion; the bond stress between epoxy coated steel rebar and concrete is reduced as compared to ordinary steel rebar, etc. In European and American countries, in order to allow the service life of structures to reach the design requirement of 100 years, stainless steel rebar is developed, and because the critical concentration causing its corrosion is increased a lot compared to ordinary steel rebar, the durability of concrete structures is greatly increased. But its cost is expensive, at about 6-10 times that of ordinary carbon steel rebar, therefore, it cannot be used for large scale application in engineering, and is normally used only at key positions of structures or in relatively harsh environments. Furthermore, macro cell corrosion easily occurs when stainless steel rebar is overlapped with ordinary steel rebar, which also adversely affect the service life of structures.

Research and development of non-rebar low alloy corrosion resistant steel is relatively mature both at home and abroad. Marine Steel is developed in U. S. in 1950s, APS20A Steel is developed in France in 1960s, and sea water corrosion resistant 10CrMoAl steel is developed in China in 1970s. Corrosion resistance performances of these steels are enhanced to a great extent compared to ordinary carbon steel, but they still cannot meet the prolonged service life required in reinforced concrete structures. Therefore, all of these types of steels cannot be used in oceanic reinforced concrete structures.

Japanese patent application JP2013-166992A discloses a corrosion resistant steel for marine structures, offshore wind power structures, bridges in the coastal area, harbour facilities, etc. The steel disclosed comprises, e.g., less than 1.0% of Mo and less than 0.01 % of rare earth metals.

Chinese patent literature CN102605255A discloses a 400MPa level corrosion resistant steel rebar comprising element ingredients of: 0.1 %-0.25% of C, 0.5%-0.90% of Si, 0.7%-1.5% of Mn, 0.04%-0.09% of P, 0.015% or less of S, 0.3%-0.6% of Cu, 0.1 %-0.4% of Ni, 0.1% of Cr, and 0.03% ∼ 0.08% of V. Its corrosion resistance performance is increased by 2 times compared to ordinary steel rebar, but the increment is still too limited to meet the service life requirement of 50-100 years for oceanic reinforced concrete structures.

### Summary of the Invention

Therefore, a technical problem to be solved by the present invention is to overcome the technical defects in prior art that steel rebar has poor corrosion resistance performance in ocean environment and cannot meet the designed service life of reinforced concrete structures, by providing a steel rebar with excellent corrosion resistance performance and comprehensive mechanical properties as well as a production method thereof.

In order to solve the above-mentioned technical problem, the present invention provides a steel rebar comprising the following ingredients calculated in weight percentage:
0.005%-0.030% of C,
0.3%-0.6% of Si,
1.2%-2.5% of Mn,
0.01% or less of P,
0.01% or less of S,
8.0%-10.0% of Cr,
1.0%-3.0% of Mo,
0.2%-0.4% of Sn,
0.01%-0.05% of Rare Earth element,
0.04%-0.18% of V and/or 0.010%-0.030% of Ti,
and the remainder being Fe and unavoidable impurities.

Preferably, there is provided a steel rebar with a 500MPa level yield strength comprising the following ingredients calculated in weight percentage:
0.005%-0.030% of C,
0.3%-0.6% of Si,
1.7%-2.5% of Mn,
0.01% or less of P,
0.01% or less of S,
8.0%-10.0% of Cr,
1.5%-2.0% of Mo,
0.2%-0.4% of Sn,
0.01%-0.05% of Rare Earth element,
0.04%-0.08% of V, and
the remainder being Fe and unavoidable impurities.

More preferably, there is provided a steel rebar with a 600MPa level yield strength comprising the following ingredients calculated in weight percentage:
0.005%-0.030% of C,
0.3%-0.6% of Si,
1.7%-2.5% of Mn,
0.01% or less of P,
0.01% or less of S,
8.0%-10.0% of Cr,
1.8%-3.0% of Mo,
0.2%-0.4% of Sn,
0.01%-0.05% of Rare Earth element,
0.10%-0.18% of V,
0.010%-0.030% of Ti, and
the remainder being Fe and unavoidable impurities.

The steel rebar has a microscopic structure composed of ferrite and bainite, with the ferrite accounting for a percentage of 50%-70%.
the steel rebar has a ratio of tensile strength to yield strength at greater than 1.25, a maximum stress total elongation percentage greater than 9%, an after-fracture elongation percentage greater than 18%, a corrosion rate by cyclic immersion corrosion test at less than 0.45m²h, and a corrosion rate by salt spray corrosion test at less than 0.45m²h.

Moreover, the present invention also provides a production method of steel rebar comprising the following steps:
S1: performing preliminary desulfurization of molten iron to control the sulfur content at no more than 0.01%;
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping;
S3: performing steel tapping, during the process of which, alloying elements of Si and Mn are added for deoxygenation and carbon powder and slag former are also added;
S4: performing refining outside the convertor, by adding Cr element and meanwhile performing decarburization by blowing oxygen in an RH vacuum refining furnace so as to control the Cr and C contents within the required range; performing deoxygenation with an LF furnace, adding the required alloying elements of Mn, Mo, Sn, Rare Earth, as well as V and/or Ti, into the steel after deoxygenation, and then adding calcium-ferrum alloy under soft stirring by blowing inert gas, so as to control contents of these elements within the required range; raising the temperature of the molten steel and adding a cover agent;
S5: performing continuous casting, by casting the molten steel under protective casting with a continuous casting machine to form a continuous casting slab;
S6: performing rolling, by heating the continuous casting slab to a temperature higher than its austenitization temperature in a heating furnace, rough rolling, moderate rolling, precision rolling, and placing the rolled steel after precision rolling onto a cooling bed for air cooling, so as to produce a finished product of steel rebar with the required ingredients.

In Step S2, the steel for steel tapping has a temperature no higher than 1690°C.

In Step S4, the decarburization by blowing oxygen is performed at a temperature no lower than 1605°C during refining in the RH vacuum refining furnace, the deoxygenation is performed at a temperature no lower than 1575°C during refining in the LF furnace to control the oxygen content at 0.002%-0.005%, the soft stirring is performed for a duration no less than 5min, and the temperature of the molten steel is raised to 1570-1600°C.

In Step S6, the continuous casting slab is heated to 1100-1200°C in the heating furnace, the temperature when the rolled steel is initially placed onto the cooling bed is 900-960°C, the start rolling temperature before the rough rolling is 1030-1100°C, and the temperature during the precision rolling is 950-1050°C.

In the steel, C is an important strengthening element mainly existing in the form of carbide to provide functions of precipitation hardening and crystal grain refining. However, C has a strong affinity with Cr, and may form a series of complicated carbides with Cr. The formation of such carbides would reduce corrosion resistance of steel at the same time of increasing hardness of steel. Furthermore, too much content of C would reduce plasticity and toughness of steel, thus deteriorating welding performance of steel.

Si is an important reducing agent and deoxidizing agent, and when added into steel, Si can significantly increase elastic limit, yield point and tensile strength of steel. When Si is combined with Mo, W, Cr, etc., it has certain function to increase corrosion resistance and oxidation resistance. But increasing the content of Si would reducing welding performance of steel.

Mn is a good deoxidizing agent and desulfurizing agent, provides a function of solid solution strengthening in steel, is an important strengthening element, and at the same time is an austenite forming element. However, too much content of Mn would significantly increase hardenability of steel, thus reducing plasticity and weldability of steel. In the aspect of corrosion resistance performance, the function of Mn is not notable.

S and P are harmful impurity elements during steelmaking process, because they easily form harmful inclusions in steel, which reduces toughness and plasticity of steel. Some weathering resistant steel adopts an ingredient design of Cu-P system. but the increment of its corrosion resistance is limited, while P easily forms segregation at grain boundaries which increases brittleness of steel. Therefore, the present invention adopts very low contents of S and P within a range no more than 0.01%.

Cr is an important element which increases oxidation resistance and corrosion resistance, and by forming a stable passive film on the steel surface under suitable environmental conditions, Cr can increase corrosion resistance performance of steel. However, the function of Cr in a non-oxidative medium is not as notable as Mo or Ni. Solely adding Cr element cannot greatly enhance sea water corrosion resistance performance of steel, but instead would increase susceptibility to pitting corrosion tendency.

Mo may generally increase corrosion resistance performance of steel, by causing passivation of the steel surface in both reductive acids and strong oxidative salt solutions, and Mo can also prevent steel from pitting corrosion in chloride solutions. When the content of Mo is relatively high (>3%), oxidation resistance of steel deteriorates. In the aspect of structure property, Mo can promote crystal grain refining and increase hardenability and heat resistance of steel.

Sn is a corrosion resistant metal which does not oxidize in air at normal temperature and, when heated intensely, stabilizes by forming stannic oxide protective film on its surface. In addition, Sn is stable towards water, can slowly dissolve in a dilute acid, and quickly dissolves in a concentrated acid. Sn is mainly used for manufacturing alloy and producing tin plates. When added as an alloying element to form a solid solution in a matrix, Sn can increase the electrode potential of the matrix, reduce the driving force of electrochemical corrosion of steel itself, lower the corrosion rate, and also cause an increasing tendency of strength and hardness of steel. When Sn interacts with Cr and Mo, they can significantly increase corrosion resistance performance of steel.

Rare Earth element may notably increase the overall corrosion resistance performance of steel when added into steel at a proper amount. The important materialogy reasons for improvement on corrosion resistance performance of steel includes the functions of Rare Earth element in purifying molten steel, metamorphic inclusions, and improving microstructure conditions and grain boundary conditions. Solid solutions of Rare Earth element in steel can increase the polarization resistance and self-corrosion potential of steel matrix, which is beneficial for increasing corrosion resistance performance of steel matrix.

Compared to prior art, the aforementioned technical solution of the present invention has the following advantages:
(1) In the steel rebar of the present invention, the content of C is controlled at 0.005%-0.030%, the content of Si is controlled at 0.3%-0.6%, the content of Mn is controlled at 1.2%-2.5%, the contents of impurity elements S and P are both controlled at no more than 0.001%, and 8.0%-10.0% of Cr, 1.0%-3.0% of Mo, 0.01%-0.05% of Rare Earth element are added, accompanied by adding 0.2%-0.4% of Sn. By providing a reasonable ratio of element ingredients, as well as interaction between Cr and Sn, the corrosion resistance performance of the steel product is significantly increased, and the added Mo and Rare Earth element improve pitting corrosion resistance and inter-granular corrosion resistance of the steel product, thereby greatly improving the sea water corrosion resistance performance of the steel rebar and increasing the service life of the steel rebar in sea water.
(2) In the steel rebar of the present invention, there contains 0.005-0.030% of C, 0.3%-0.6% of Si, 1.2%-1.8% of Mn, 0.01% or less of P, 0.01% or less of S, 8.0%-10.0% of Cr, 1.0%-1.6% of Mo, 0.2%-0.4% of Sn, 0.01%-0.05% of Rare Earth element, and the remainder being Fe and unavoidable impurities. By providing a reasonable ingredient design, a 400MPa level corrosion resistant steel rebar is produced, so as to obtain a steel rebar which is low-cost, able to meet requirements of basic mechanical properties, and resistant to sea water corrosion.
(3) In the steel rebar of the present invention, there contains 0.005%-0.030% of C, 0.3%-0.6% of Si, 1.2%-2.5% of Mn, 0.01% or less of P, 0.01% or less of S, 8.0%-10.0% of Cr, 1.0%-3.0% of Mo, 0.2%-0.4% of Sn, 0.01%-0.05% of Rare Earth element, 0.04%-0.18% of V and/or 0.010%-0.030% of Ti, and the remainder being Fe and unavoidable impurities. Micro-alloying elements V and/or Ti are further added into steel. V is a micro-alloying element that can cause a V(C,N) compound to precipitate out during the rolling process, which prevents austenite and ferrite form growing and has relatively strong effects of precipitation strengthening and refined crystalline strengthening as well as certain effect of solid solution strengthening, thereby significantly increase the strength of steel and thus compensating for the defect of insufficient strength due to low carbon content. Ti is a strong forming element of carbonitride with effects of refining crystal grain structure and precipitation strengthening. Meanwhile, because carbon preferentially reacts with Ti to produce carbon titanium compounds, the precipitation of chromium carbide in chromium-containing steel which causes chromium depletion at grain boundaries is avoided, thereby effectively preventing inter-granular corrosion. By solid solution strengthening, refined crystalline strengthening, and precipitation strengthening as V(C,N) and/or Ti(C,N) are produced, the micro-alloying elements V and/or Ti increase the strength of steel and endow the steel rebar with excellent mechanical properties.
(4) In the steel rebar of the present invention, by controlling the element contents in steel, especially the contents of micro-alloying elements V and/or Ti, steel products that meet various strength requirements are produced. For instance, in a steel rebar with a 500MPa level yield strength, there contains 0.005%-0.030% of C, 0.3%-0.6% of Si, 1.7%-2.5% of Mn, 0.01% or less of P, 0.01% or less of S, 8.0%-10.0% of Cr, 1.5%-2.0% of Mo, 0.2%-0.4% of Sn, 0.01%-0.05% of Rare Earth element, 0.04%-0.08% of V, and the remainder being Fe and unavoidable impurities; for another instance, in a steel rebar with a 600MPa level yield strength, there contains 0.005%-0.030% of C, 0.3%-0.6% of Si, 1.7%-2.5% of Mn, 0.01% or less of P, 0.01% or less of S, 8.0%-10.0% of Cr, 1.8%-3.0% of Mo, 0.2%-0.4% of Sn, 0.01%-0.05% of Rare Earth element, 0.10%-0.18% of V, 0.010%-0.030% of Ti, and the remainder being Fe and unavoidable impurities.
(5) In the steel rebar of the present invention, the percentage of ferrite is 50%-70%. While bainite has good strength and toughness, ferrite has better plasticity. By reasonably controlling a ratio of the two phases, the steel rebar can be endowed with excellent comprehensive mechanical properties, wherein, on the basis of obtaining the required yield strength and tensile strength, the after-fracture elongation percentage is greater than 18%, the ratio of tensile strength to yield strength is greater than 1.25, and the maximum stress total elongation percentage is greater than 9%, thereby endowing the steel product with good anti-knock performance.
(6) The production method of steel rebar of the present invention controls the content of S by a KR desulfurization method, controls the content of P in a convertor, adds alloying elements of Si and Mn during the steel tapping process for deoxygenation and meanwhile adds carbon powder and slag former to create a reductive atmosphere for the refining furnace, carries out decarburization by blowing oxygen in an RH vacuum refining furnace so as to control the contents of carbon and chromium elements, carries out deoxygenation in an LF furnace while adding the remaining alloying elements into steel so as to control the contents of oxygen and various alloying elements, as well as adding calcium-ferrum alloy to perform denaturation treatment on the inclusions, carries out soft stirring to make the ingredients uniformly distributed and remove inclusions, provides protective casting during the continuous casting process so as to control the gas content in steel, to prevent oxidization or secondary inclusions, heats the casting slab to 1100-1200°C before rolling in a heating furnace to ensure austenization and cause the elements therein to sufficiently enter a solid solution state, adopts rough rolling, moderate rolling and precision rolling during rolling can strictly control the deformation amount of the steel when rolled, while the precipitation strengthening effect of micro-alloying elements V(C,N) and/or Ti(C,N) can be brought into full play by controlling the rolling parameters, and places the rolled steel onto a cooling bed for air cooling so as to render the final microstructure of the steel product being bainite and ferrite.
(7) The production method of steel rebar of the present invention, by controlling the temperature of the steel for steel tapping at no higher than 1690°C, reduces the oxygen content in the steel, increases the element yield, reduces inclusions in the steel, increases the service life of the convertor, increases the quality of steel, and reduces production cost of steel.
(8) In the production method of steel rebar of the present invention, by controlling the temperature of decarburization by blowing oxygen during refining in the RH vacuum refining furnace to be no lower than 1605°C, the decarburization effect in the RH furnace can be increased, and it also facilitates controlling the contents of carbon and chromium elements in the steel. By controlling the temperature of deoxygenation during refining in the LF furnace, the refinement effect of deoxygenation in the LF furnace can be increased, which facilitates controlling the oxygen content within a predetermined range. And by controlling the oxygen content at 0.002%-0.005% through deoxygenation in the LF furnace, inclusions in the steel can be effectively controlled, and the quality of the steel in improved. By controlling the duration of soft stirring at no less than 5min, the ingredients and temperature of steel can be made more uniformly distributed, and it also facilitates removing the inclusions by floating. By raising the temperature of the molten steel to 1570-1600°C before continuous casting, smooth operation of the continuous casting is ensured.
(9) In the production method of steel rebar of the present invention, by heating the casting slab to 1100-1200°C in the heating furnace, the steel is heated to a temperature higher than its austenitization temperature, and a solid solution state of the alloying elements in the steel is ensured. By controlling the start rolling temperature at 1030-1100°C and controlling the temperature during the precision rolling at 950-1050°C, precipitation of a strengthening phase can be induced by deformation, so as to increase the strength of the steel. By controlling the temperature when the steel product is initially placed onto the cooling bed, the required microstructure of bainite plus ferrite can be obtained.
(10) The production method of steel rebar of the present invention, by accurately controlling the element contents and temperature of the molten steel during each procedure, greatly reduces the amount of harmful elements and inclusions in the steel, and improves the quality, mechanical properties and corrosion resistance performance of the steel.
(11) The steel rebar manufactured by using the steel rebar production method of the present invention, by means of reasonable processing steps, has a microscopic structure composed of ferrite and bainite, with the ferrite accounting for a percentage of 50%-70%. While bainite has good strength and toughness, ferrite has better plasticity. By reasonably controlling a ratio of the two phases, the steel rebar can be endowed with excellent comprehensive mechanical properties, wherein, on the basis of obtaining the required yield strength and tensile strength, the after-fracture elongation percentage is greater than 18%, the ratio of tensile strength to yield strength is greater than 1.25, and the maximum stress total elongation percentage is greater than 9%, thereby endowing the steel product with good anti-knock performance

### Brief Description of the Drawings

In order to make the present invention easy and clear to understand, hereinafter, the present invention will be further described in detail according to specific embodiments of the present invention and with reference to the appended drawings, wherein:
FIG. 1 is a microstructure view of a steel rebar of the present invention.

### Detailed Description of Embodiments

**Table 1 Steel rebar ingredients of Embodiments 4-10 as well as comparison examples 1-3 wt.%**

| | C | Si | Mn | Cr | Mo | RE | Sn | V | Ti | P | S |
|---|---|---|---|---|---|---|---|---|---|---|---|
| Embodiment 4 | 0.020 | 0.5 | 2.3 | 8.5 | 2.2 | 0.02 | 0.25 | 0.04 | - | <0.01 | <0.01 |
| Embodiment 5 | 0.025 | 0.55 | 1.7 | 8.2 | 2.3 | 0.02 | 0.35 | 0.18 | 0.01 | <0.01 | <0.01 |
| Embodiment 6 | 0.009 | 0.35 | 1.8 | 8.5 | 2.5 | 0.04 | 0.36 | 0.1 | 0.03 | <0.01 | <0.01 |
| Embodiment 7 | 0.012 | 0.40 | 2.2 | 9.5 | 1.5 | 0.03 | 0.28 | - | 0.02 | <0.01 | <0.01 |
| Embodiment 8 | 0.012 | 0.57 | 1.8 | 9.7 | 2.0 | 0.03 | 0.21 | 0.08 | - | <0.01 | <0.01 |
| Embodiment 9 | 0.018 | 0.50 | 1.9 | 9.0 | 1.7 | 0.02 | 0.30 | 0.06 | - | <0.01 | <0.01 |
| Embodiment 10 | 0.026 | 0.50 | 2.3 | 8.1 | 1.8 | 0.05 | 0.40 | 0.15 | 0.02 | <0.01 | <0.01 |
| Comparison Example 1 | 0.23 | 0.54 | 1.5 | - | - | - | - | - | - | <0.01 | <0.01 |
| Comparison Example 2 | 0.015 | 0.48 | 1.9 | 9.1 | 1.8 | 0.02 | 0.60 | - | - | <0.01 | <0.01 |
| Comparison Example 3 | 0.024 | 0.52 | 2.0 | 9.8 | 2.0 | 0.02 | - | - | - | <0.01 | <0.01 |

### Embodiment 4

The present embodiment provides a steel rebar, comprising the following elements: C, Si, Mn, P, S, Cr, Mo, Sn, Rare Earth element, V, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1690°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, performed by adding Cr element and meanwhile performing decarburization by blowing oxygen at 1620°C in an RH vacuum refining furnace, so that C element is partially removed by the decarburization process, thereby controlling the contents of Cr and C elements within the required range; performing deoxygenation with an LF furnace at 1590°C until the oxygen content in the molten steel reaches 20ppm, and adding the required alloying elements of Mn, Mo, Sn, Rare Earth, V into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 6min to make the ingredients and temperature of the steel uniformly distributed and to facilitate the removal of inclusions by floating, so that the contents of the ingredients are controlled within the ranges as shown in data of Embodiment 4 in Table 1; raising the temperature of the molten steel to 1585°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1180°C in a heating furnace, performing rough rolling, moderate rolling and precision rolling by using a continuous rod and wire rolling machine with the start rolling temperature at 1040°C and the precision rolling temperature at 990°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 950°C. By means of the technique of controlled rolling and controlled cooling, the microstructure of bainite plus ferrite is finally obtained.

### Embodiment 5

The present embodiment provides a steel rebar, comprising the following elements: C, Si, Mn, P, S, Cr, Mo, Sn, Rare Earth element, V, Ti, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1675°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, by adding Cr element and meanwhile performing decarburization by blowing oxygen at 1615°C in an RH vacuum refining furnace, so that C element is partially removed by the decarburization process, thereby controlling the contents of Cr and C elements within the required range; performing deoxygenation with an LF furnace at 1580°C until the oxygen content in the molten steel reaches 25ppm, and adding the required alloying elements of Mn, Mo, Sn, Rare Earth, V, Ti into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 7min to make the ingredients and temperature of the steel uniformly distributed and to facilitate the removal of inclusions by floating, so that the contents of the ingredients are controlled within the ranges as shown in data of Embodiment 5 in Table 1; raising the temperature of the molten steel to 1580°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1190°C in a heating furnace, performing rough rolling, moderate rolling and precision rolling by using a continuous rod and wire rolling machine with the start rolling temperature at 1095°C and the precision rolling temperature at 1030°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 950°C. By means of the technique of controlled rolling and controlled cooling, the microstructure of bainite plus ferrite is finally obtained.

### Embodiment 6

The present embodiment provides a steel rebar, comprising the following elements: C, Si, Mn, P, S, Cr, Mo, Sn, Rare Earth element, V, Ti, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1670°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, by adding Cr element and meanwhile performing decarburization by blowing oxygen at 1610°C in an RH vacuum refining furnace, so that C element is partially removed by the decarburization process, thereby controlling the contents of Cr and C elements within the required range; performing deoxygenation with an LF furnace at 1580°C until the oxygen content in the molten steel reaches 20ppm, and adding the required alloying elements of Mn, Mo, Sn, Rare Earth, V, Ti into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 7min to make the ingredients and temperature of the steel uniformly distributed and to facilitate the removal of inclusions by floating, so that the contents of the ingredients are controlled within the ranges as shown in data of Embodiment 6 in Table 1; raising the temperature of the molten steel to 1590°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1185°C in a heating furnace, performing rough rolling, moderate rolling and precision rolling by using a continuous rod and wire rolling machine with the start rolling temperature at 1085°C and the precision rolling temperature at 1035°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 955°C. By means of the technique of controlled rolling and controlled cooling, the microstructure of bainite plus ferrite is finally obtained.

### Embodiment 7

The present embodiment provides a steel rebar, comprising the following elements: C, Si, Mn, P, S, Cr, Mo, Sn, Rare Earth element, Ti, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1685°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, by adding Cr element and meanwhile performing decarburization by blowing oxygen at 1615°C in an RH vacuum refining furnace, so that C element is partially removed by the decarburization process, thereby controlling the contents of Cr and C elements within the required range; performing deoxygenation with an LF furnace at 1580°C until the oxygen content in the molten steel reaches 20ppm, and adding the required alloying elements of Mn, Mo, Sn, Rare Earth, Ti into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 7min to make the ingredients and temperature of the steel uniformly distributed and to facilitate the removal of inclusions by floating, so that the contents of the ingredients are controlled within the ranges as shown in data of Embodiment 7 in Table 1; raising the temperature of the molten steel to 1585°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1180°C in a heating furnace, performing rough rolling, moderate rolling and precision rolling by using a continuous rod and wire rolling machine with the start rolling temperature at 1080°C and the precision rolling temperature at 1020°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 940°C. By means of the technique of controlled rolling and controlled cooling, the microstructure of bainite plus ferrite is finally obtained.

### Embodiment 8

The present embodiment provides a steel rebar, comprising the following elements: C, Si, Mn, P, S, Cr, Mo, Sn, Rare Earth element, V, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1680°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, by adding Cr element and meanwhile performing decarburization by blowing oxygen at 1610°C in an RH vacuum refining furnace, so that C element is partially removed by the decarburization process, thereby controlling the contents of Cr and C elements within the required range; performing deoxygenation with an LF furnace at 1585°C until the oxygen content in the molten steel reaches 20ppm, and adding the required alloying elements of Mn, Mo, Sn, Rare Earth, V into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 7min to make the ingredients and temperature of the steel uniformly distributed and to facilitate the removal of inclusions by floating, so that the contents of the ingredients are controlled within the ranges as shown in data of Embodiment 8 in Table 1; raising the temperature of the molten steel to 1590°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1150°C in a heating furnace, performing rough rolling, moderate rolling and precision rolling by using a continuous rod and wire rolling machine with the start rolling temperature at 1065°C and the precision rolling temperature at 1025°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 965°C. By means of the technique of controlled rolling and controlled cooling, the microstructure of bainite plus ferrite is finally obtained.

### Embodiment 9

The present embodiment provides a steel rebar, comprising the following elements: C, Si, Mn, P, S, Cr, Mo, Sn, Rare Earth element, V, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1675°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, by adding Cr element and meanwhile performing decarburization by blowing oxygen at 1605°C in an RH vacuum refining furnace, so that C element is partially removed by the decarburization process, thereby controlling the contents of Cr and C elements within the required range; performing deoxygenation with an LF furnace at 1575°C until the oxygen content in the molten steel reaches 20ppm, and adding the required alloying elements of Mn, Mo, Sn, Rare Earth, V into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 7min to make the ingredients and temperature of the steel uniformly distributed and to facilitate the removal of inclusions by floating, so that the contents of the ingredients are controlled within the ranges as shown in data of Embodiment 9 in Table 1; raising the temperature of the molten steel to 1580°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1105°C in a heating furnace, performing rough rolling, moderate rolling and precision rolling by using a continuous rod and wire rolling machine with the start rolling temperature at 1045°C and the precision rolling temperature at 1005°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 945°C. By means of the technique of controlled rolling and controlled cooling, the microstructure of bainite plus ferrite is finally obtained.

### Embodiment 10

The present embodiment provides a steel rebar, comprising the following elements: C, Si, Mn, P, S, Cr, Mo, Sn, Rare Earth element, V, Ti, Fe and unavoidable impurities, wherein, the weight percentages of the ingredients are as shown in Table 1, the mechanical properties are as shown in Table 2, and the corrosion resistance performance is as shown in Table 3.

The present embodiment also provides a production method of steel rebar comprising the following steps:
S1: performing preliminary desulfurization of molten iron by using a KR method to control the sulfur content at no more than 0.01%. Because sulfur element as an impurity element would reduce mechanical properties and corrosion resistance performance of steel and normally cannot be removed in a convertor, therefore, in order to reduce the sulfur content in steel, preliminary desulfurization treatment needs to be performed in molten iron. Before performing desulfurization, the blast furnace slag needs to be removed in order to increase the desulfurization efficiency. A mixture of lime powder and fluorite mixed at a mass ratio of 9:1 is adopted as the desulfurization agent. After still standing of the desulfurated molten iron, the desulfurization residue is removed to prevent it from entering the convertor and causing convertor resulfurization. Thereby, the sulfur content in the steel is ensured to be controlled at less than 0.01%.
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping. The convertor is a top and bottom combined blown converter.
S3: performing steel tapping with a steel tapping temperature of 1685°C. During the steel tapping process, alloying elements of Si and Mn are added for deoxygenation, and carbon powder and slag former are also added. During the operation process of steel tapping, a protective gas is blown into the molten steel for stirring the molten steel at a pressure of 0.5MPa. The fluidity of the molten steel is utilized to make the deoxygenation of the added Si and Mn elements more thoroughly and to facilitate the removal of inclusions by floating. The carbon powder and slag former are added to increase the carbon content of steel and to produce reduced slag, so as to prepare for the subsequent refining procedure outside the convertor.
S4: performing refining outside the convertor, by adding Cr element and meanwhile performing decarburization by blowing oxygen at 1620°C in an RH vacuum refining furnace, so that C element is partially removed by the decarburization process, thereby controlling the contents of Cr and C elements within the required range; performing deoxygenation with an LF furnace at 1585°C until the oxygen content in the molten steel reaches 20ppm, and adding the required alloying elements of Mn, Mo, Sn, Rare Earth, V, Ti into the steel after deoxygenation, wherein, while the added alloying elements may be a pure metallic element, normally they are added in the form of iron alloy; and then adding calcium-ferrum alloy to perform denaturation treatment on the inclusions, performing soft stirring by blowing inert gas for 7min to make the ingredients and temperature of the steel uniformly distributed and to facilitate the removal of inclusions by floating, so that the contents of the ingredients are controlled within the ranges as shown in data of Embodiment 10 in Table 1; raising the temperature of the molten steel to 1595°C during a later period of processing with the LF furnace, in order to ensure smooth operation of continuous casting, and then adding a cover agent which usually is carbonized rice husk.
S5: continuous casting, by casting the molten steel under protective casting with a continuous casting machine to produce small square billets of 150mm×150mm.
S6: performing rolling, by heating the continuous casting slab to 1195°C in a heating furnace, performing rough rolling, moderate rolling and precision rolling by using a continuous rod and wire rolling machine with the start rolling temperature at 1095°C and the precision rolling temperature at 1045°C, without passing water cooling after precision rolling, and placing the rolled steel after precision rolling onto a cooling bed for air cooling until room temperature, thereby producing a finished product of steel rebar as shown in Table 1, wherein, the temperature when the rolled steel is initially placed onto the cooling bed is 955°C. By means of the technique of controlled rolling and controlled cooling, the microstructure of bainite plus ferrite is finally obtained.

### Experimental Example

In order to prove the technical effects of the present invention, the following experiments are performed on the steel rebar produced by Embodiment 4-10 and comparison examples 1-3:

### 1. Experimental methods

1.1 mechanical property tests: performed according to "GB1499.2-2007, steel used in reinforced concrete, Part II: hot-rolled ribbed rebar". The yield strength (R_{0.2}), tensile strength (Rₘ), and after-fracture elongation percentage (A) are tested.
1.2 corrosion resistance performance tests:
   1.2.1 cyclic immersion corrosion test: performed according to "corrosion test methods of steel rebar in a chloride ion environment, a draft for consultation" proposed by Steel Industry Association of China and drafted by institutes of Iron and Steel Research Institute and Metallurgical Industry Information Standardization Research Institute.
      The test sample is a cylinder of ∮13mm×50mm;
      The test solution is a solution of sodium chloride with an initial concentration of (0.34±0.009)mol•L⁻¹ (an initial mass percentage of 2.0%±0.05%). And the specific test conditions are as follows:
      Temperature: 45°C±2°C
      Humidity: 70%±10% RH
      PH value of solution: 6.5-7.2
      Test time: 360h
      Each cyclic period: 60 min±5min, with an immersion time of 12 min±2min
      Highest temperature of test sample surface after baking: 70°C±10°C
   1.2.2 salt spray corrosion test: performed according to "GBT10125-1997, corrosion tests in an artificial atmosphere, salt spray test".
      The test sample is a test plate of 3mm×15mm×40mm;
      The test solution is a solution of sodium chloride with a concentration of (50±5)g•L⁻¹ (a mass percentage of 5.0%±0.5%). And the specific test conditions are as follows:
      Temperature: 35°C±2°C
      PH value of solution: 6.5-7.2
      Test time: 360h

### 2. Experimental results

Table 2 shows the effects about mechanical properties of Embodiment 4-10 and comparison examples 1-3. Table 3 shows the effects about corrosion resistance performance of Embodiment 4-10 and comparison examples 1-3.

**Table 2 Effects about mechanical properties**

| | R_{0.2}/MPa | Rₘ/MPa | A/% | Rₘ/ R_{0.2} | A_{gt}/% |
|---|---|---|---|---|---|
| Embodiment 4 | 561 | 728 | 18.9 | 1.30 | 10.8 |
| Embodiment 5 | 611 | 793 | 19.6 | 1.29 | 10.5 |
| Embodiment 6 | 554 | 755 | 20.8 | 1.36 | 10.3 |
| Embodiment 7 | 524 | 716 | 21.2 | 1.37 | 10.7 |
| Embodiment 8 | 523 | 743 | 25.0 | 1.42 | 11.3 |
| Embodiment 9 | 536 | 729 | 21.0 | 1.36 | 10.7 |
| Embodiment 10 | 621 | 795 | 18.0 | 1.28 | 9.5 |
| Comparison Example 1 | 435 | 632 | 22.0 | 1.45 | 12.0 |
| Comparison Example 2 | 486 | 586 | 13.4 | 1.21 | 6.2 |
| Comparison Example 3 | 477 | 687 | 24.8 | 1.44 | 11.0 |

**Table 3 Effects about corrosion resistance performance**

| | cyclic immersion test | | | salt spray test | | |
|---|---|---|---|---|---|---|
| | Corrosion rate (g/m²·h) | Relative corrosion rate | Increase of corrosion resistance performance (%) | Corrosion rate (g/m²·h) | Relative corrosion rate | Increase of corrosion resistance performance (%) |
| Embodiment 4 | 0.356 | 0.109 | 821 | 0.367 | 0.117 | 758 |
| Embodiment 5 | 0.441 | 0.135 | 643 | 0.445 | 0.141 | 608 |
| Embodiment 6 | 0.349 | 0.106 | 839 | 0.360 | 0.114 | 775 |
| Embodiment 7 | 0.386 | 0.118 | 749 | 0.395 | 0.125 | 697 |
| Embodiment 8 | 0.272 | 0.083 | 1105 | 0.288 | 0.091 | 994 |
| Embodiment 9 | 0.370 | 0.113 | 786 | 0.381 | 0.121 | 727 |
| Embodiment 10 | 0.433 | 0.132 | 657 | 0.435 | 0.138 | 624 |
| Comparison Example 1 | 3.278 | 1 | - | 3.150 | 1 | - |
| Comparison Example 2 | 0.365 | 0.111 | 798 | 0.377 | 0.120 | 736 |
| Comparison Example 3 | 0.456 | 0.151 | 561 | 0.463 | 0.160 | 526 |

(The relative corrosion rates in Table 3 are all compared with Comparison Example 1, by setting the relative corrosion rate of Comparison Example 1 to be 1.000)

As known from Table 3, in Embodiment 4-10, because Cr, Sn, Mo, Rare Earth elements are added, the corrosion resistance performance of steel rebar is increased by more than 600% compared with Comparison Example 1. As can be seen from the corrosion resistance performance data of Comparison Example 3, the increment of the corrosion resistance performance of steel rebar which does not contain Sn element is not as great as that of steel rebar which contains Sn element. In Embodiments 4-10, V and/or Ti elements are added into steel rebar, and it can be seen from Table 2, the adding of V and/or Ti elements improves the yield strength and tensile strength of steel rebar, and at the same time, the after-fracture elongation percentage is greater than 18%, the ratio of tensile strength to yield strength is greater than 1.25, and the maximum stress total elongation percentage is greater than 9%, thereby endowing the steel product with good anti-knock performance.

In the steel rebar of the present invention, by reasonably designing the ingredients and accurately controlling the element ingredients and temperature during the smelting process, in combination with the technique of controlled rolling and controlled cooling, the steel rebar is made to obtain a microstructure of bainite plus ferrite (with the ferrite accounting for a percentage of 50%-70%) as shown in FIG. 1, thereby endowing the steel rebar with excellent comprehensive mechanical properties as well as excellent corrosion resistance performance which is increased by more than 6 times compared to ordinary steel rebar, so that the service life requirement of reinforced concrete structures in oceanographic engineering can be fulfilled.

Apparently, the aforementioned embodiments are merely examples illustrated for clearly describing the present invention, rather than limiting the implementation ways thereof. For those skilled in the art, various changes and modifications in other different forms can be made on the basis of the aforementioned description. It is unnecessary and impossible to exhaustively list all the implementation ways herein. However, any obvious changes or modifications derived from the aforementioned description are intended to be embraced within the protection scope of the present invention.

## Claims

1. A steel rebar, **characterized in** comprising the following ingredients calculated in weight percentage:
0.005%-0.030% of C,
0.3%-0.6% of Si,
1.2%-2.5% of Mn,
0.01% or less of P,
0.01% or less of S,
8.0%-10.0% of Cr,
1.0%-3.0% of Mo,
0.2%-0.4% of Sn,
0.01%-0.05% of Rare Earth element,
0.04%-0.18% of V and/or 0.010%-0.030% of Ti,
and the remainder being Fe and unavoidable impurities.

2. The steel rebar in accordance with Claim 1, **characterized in** comprising the following ingredients calculated in weight percentage:
0.005%-0.030% of C,
0.3%-0.6% of Si,
1.7%-2.5% of Mn,
0.01% or less of P,
0.01% or less of S,
8.0%-10.0% of Cr,
1.5%-2.0% of Mo,
0.2%-0.4% of Sn,
0.01%-0.05% of Rare Earth element,
0.04%-0.08% of V, and
the remainder being Fe and unavoidable impurities.

3. The steel rebar in accordance with Claim 1, **characterized in** comprising the following ingredients calculated in weight percentage:
0.005%-0.030% of C,
0.3%-0.6% of Si,
1.7%-2.5% of Mn,
0.01% or less of P,
0.01% or less of S,
8.0%-10.0% of Cr,
1.8%-3.0% of Mo,
0.2%-0.4% of Sn,
0.01%-0.05% of Rare Earth element,
0.10%-0.18% of V,
0.010%-0.030% of Ti, and
the remainder being Fe and unavoidable impurities.

4. The steel rebar in accordance with any one of Claims 1-3, **characterized in that**, the steel rebar has a microscopic structure composed of ferrite and bainite, with the ferrite accounting for a percentage of 50%-70%.

5. The steel rebar in accordance with any one of Claims 1-4, **characterized in that**,
the steel rebar has a ratio of tensile strength to yield strength at greater than 1.25, a maximum stress total elongation percentage greater than 9% and an after-fracture elongation percentage greater than 18% measured according to GB1499.2-2007;
the steel rebar has a corrosion rate by cyclic immersion corrosion test at less than 0.45m²h, and a corrosion rate by salt spray corrosion test at less than 0.45m²h measured according to GBT10125-1997.

6. A production method of steel rebar, **characterized in** comprising the following steps:
S1: performing preliminary desulfurization of molten iron to control the sulfur content at no more than 0.01%;
S2: performing smelting in a convertor, by feeding the molten iron processed by Step S1 together with steel scrap and/or pig iron into a convertor to be smelted, thus obtaining steel with a carbon content less than 0.05% and a phosphorus content less than 0.01% for steel tapping;
S3: performing steel tapping, during the process of which, alloying elements of Si and Mn are added for deoxygenation and carbon powder and slag former are also added;
S4: performing refining outside the convertor, by adding Cr element and meanwhile performing decarburization by blowing oxygen in an RH vacuum refining furnace so as to control the Cr and C contents within the range in accordance with any one of Claims 1-3; carrying out deoxygenation with an LF furnace, adding the required alloying elements of Mn, Mo, Sn, Rare Earth, as well as V and/or Ti, into the steel after deoxygenation, and then adding calcium-ferrum alloy under soft stirring by blowing inert gas, so as to control contents of these elements within the range in accordance with any one of Claims 1-3; raising the temperature of the molten steel and adding a cover agent;
S5: performing continuous casting, by casting the molten steel under protective casting with a continuous casting machine to form a continuous casting slab;
S6: performing rolling, by heating the continuous casting slab to a temperature higher than its austenitization temperature in a heating furnace, rough rolling, moderate rolling, precision rolling, and placing the rolled steel after precision rolling onto a cooling bed for air cooling, so as to produce a finished product of steel rebar with ingredients in accordance with any one of Claims 1-3.

7. The production method in accordance with Claim 6, **characterized in that**, in Step S2, the steel for steel tapping has a temperature no higher than 1690°C.

8. The production method in accordance with Claim 6 or 7, **characterized in that**, in Step S3, a protective gas is blown into the molten steel for stirring during the process of steel tapping.

9. The production method in accordance with any one of Claims 6-8, **characterized in that**, in Step S4, the decarburization by blowing oxygen is performed at a temperature no lower than 1605°C during refining in the RH vacuum refining furnace, the deoxygenation is performed at a temperature no lower than 1575°C during refining in the LF furnace to control the oxygen content at no more than 50ppm, the soft stirring is performed for a duration no less than 5min, and the temperature of the molten steel is raised to 1570-1600°C.

10. The production method in accordance with any one of Claims 6-9, **characterized in that**, in Step S6, the continuous casting slab is heated to 1100-1200°C in the heating furnace, the start rolling temperature before the rough rolling is 1030-1100°C, the temperature during the precision rolling is 950-1050°C, and the temperature when the rolled steel is initially placed onto the cooling bed is 900-960°C.

## Patentansprüche

1. Bewehrungsstahl, **dadurch gekennzeichnet, dass** er folgende Bestandteile, berechnet in Gewichtsprozent, umfasst:
0,005 % bis 0,030 % C,
0,3 % bis 0,6 % Si,
1,2 % bis 2,5 % Mn,
0,01 % oder weniger P,
0,01 % oder weniger S,
8,0 % bis 10,0 % Cr,
1,0 % bis 3,0 % Mo,
0,2 % bis 0,4 % Sn,
0,01 % bis 0,05 % Seltenerdelement,
0,04 % bis 0,18 % V und/oder 0,010 % bis 0,030 % Ti,
und als Rest Fe und unvermeidbare Verunreinigungen.

2. Bewehrungsstahl gemäß Anspruch 1, **dadurch gekennzeichnet, dass** er folgende Bestandteile, berechnet in Gewichtsprozent, umfasst:
0,005 % bis 0,030 % C,
0,3 % bis 0,6 % Si,
1,7 % bis 2,5 % Mn,
0,01 % oder weniger P,
0,01 % oder weniger S,
8,0 % bis 10,0 % Cr,
1,5 % bis 2,0 % Mo,
0,2 % bis 0,4 % Sn,
0,01 % bis 0,05 % Seltenerdelement,
0,04 % bis 0,08 % V und
als Rest Fe und unvermeidbare Verunreinigungen.

3. Bewehrungsstahl gemäß Anspruch 1, **dadurch gekennzeichnet, dass** er folgende Bestandteile, berechnet in Gewichtsprozent, umfasst:
0,005 % bis 0,030 % C,
0,3 % bis 0,6 % Si,
1,7 % bis 2,5 % Mn,
0,01 % oder weniger P,
0,01 % oder weniger S,
8,0 % bis 10,0 % Cr,
1,8 % bis 3,0 % Mo,
0,2 % bis 0,4 % Sn,
0,01 % bis 0,05 % Seltenerdelement,
0,10 % bis 0,18 % V,
0,010 % bis 0,030 % Ti und
als Rest Fe und unvermeidbare Verunreinigungen.

4. Bewehrungsstahl gemäß einem der Ansprüche 1-3, **dadurch gekennzeichnet, dass** der Bewehrungsstahl eine mikroskopische Struktur aufweist die aus Ferrit und Bainit zusammengesetzt ist, wobei der Ferrit einen Anteil von 50 % bis 70 % bildet.

5. Bewehrungsstahl gemäß einem der Ansprüche 1-4, **dadurch gekennzeichnet, dass**
der Bewehrungsstahl ein Verhältnis von Zugfestigkeit zu Streckgrenze von größer als 1,25, eine prozentuelle Gesamtdehnung bei Maximalspannung von größer als 9 % und eine prozentuelle Dehnung nach dem Bruch von größer als 18 %, gemessen gemäß GB1499.2-2007, aufweist;
der Bewehrungsstahl eine Korrosionsrate bei einer zyklischen Immersionskorrosionsprüfung von weniger als 0,45 m²h und eine Korrosionsrate bei einer Salzsprühkorrosionsprüfung von weniger als 0,45 m²h, gemessen gemäß GBT10125-1997, aufweist.

6. Verfahren zur Herstellung von Bewehrungsstahl, **dadurch gekennzeichnet, dass** es folgende Schritte umfasst:
S1: Durchführen einer vorausgehenden Entschwefelung von geschmolzenem Eisen, um den Schwefelgehalt auf nicht mehr als 0,01 % zu steuern;
S2: Durchführen von Einschmelzen in einem Konverter durch Zuführen des bei Schritt S1 verarbeiteten geschmolzenen Eisens zusammen mit Stahlschrott und/oder Roheisen in einen Konverter zum Schmelzen, um Stahl mit einem Kohlenstoffgehalt von weniger als 0,05 % und einem Phosphorgehalt von weniger als 0,01 % zum Stahlabstich zu erhalten;
S3: Durchführen von Stahlabstich, wobei während dieses Vorgangs Legierungselemente Si und Mn zur Desoxygenierung zugegeben werden und ferner Kohlenstoffpulver und Schlackenbildner zugegeben werden;
S4: Durchführen von Frischen außerhalb des Konverters durch Zugeben von Cr-Element und gleichzeitig Durchführen von Entkohlung durch Einblasen von Sauerstoff in einem RH-Unterdruck-Frischofen, um den Cr- und C-Gehalt auf den Bereich gemäß einem der Ansprüche 1-3 zu steuern; Durchführen von Desoxygenierung mit einem LF-Ofen, Zugeben der benötigten Legierungselemente Mn, Mo, Sn, Seltenerdelement sowie V und/oder Ti in den Stahl nach der Desoxygenierung und dann Zugeben von Ferrocalcium-Legierung unter leichtem Rühren durch Einblasen von Inertgas, um den Gehalt an diesen Elementen auf den Bereich gemäß einem der Ansprüche 1-3 zu steuern; Erhöhen der Temperatur des geschmolzenen Stahls und Zugeben eines Abdeckmittels;
S5: Durchführen von kontinuierlichem Gießen durch Gießen des geschmolzenen Stahls unter Schutzgießen mithilfe einer kontinuierlichen Gießanlage, um einen kontinuierlichen Gussstrang zu bilden;
S6: Durchführen von Walzen durch Erhitzen des kontinuierlichen Gussstrangs auf eine Temperatur von höher als seine Austenitisierungstemperatur in einem Heizofen, Vorwalzen, Zwischenwalzen, Präzisionswalzen und Anordnen des gewalzten Stahls nach dem Präzisionswalzen auf einem Kühlbett zur Luftkühlung, um ein fertiges Produkt aus Bewehrungsstahl mit Bestandteilen gemäß einem der Ansprüche 1-3 zu erhalten.

7. Herstellungsverfahren gemäß Anspruch 6, **dadurch gekennzeichnet, dass** bei Schritt S2 der Stahl für den Stahlabstich eine Temperatur von nicht höher als 1690 °C aufweist.

8. Herstellungsverfahren gemäß Anspruch 6 bis 7, **dadurch gekennzeichnet, dass** bei Schritt S3 zum Rühren während des Vorgangs des Stahlabstichs ein Schutzgas in den geschmolzenen Stahl geblasen wird.

9. Herstellungsverfahren gemäß einem der Ansprüche 6-8, **dadurch gekennzeichnet, dass** bei Schritt S4 die Entkohlung durch Einblasen von Sauerstoff bei einer Temperatur von nicht unter 1605 °C während des Frischens in dem RH-Unterdruck-Frischofen durchgeführt wird, die Desoxygenierung bei einer Temperatur von nicht unter 1575 °C während des Frischens in dem LF-Ofen durchgeführt wird, um den Sauerstoffgehalt auf nicht mehr als 50 ppm zu steuern, das leichte Rühren mit einer Dauer von nicht weniger als 5 min durchgeführt wird und die Temperatur des geschmolzenen Stahls auf 1570-1600 °C erhöht wird.

10. Herstellungsverfahren gemäß einem der Ansprüche 6-9, **dadurch gekennzeichnet, dass** bei Schritt S6 der kontinuierliche Gussstrang in dem Heizofen auf 1100-1200 °C erhitzt wird, die Anfangs-Walztemperatur von dem Vorwalzen 1030-1100 °C beträgt, die Temperatur während des Präzisionswalzens 950-1050 °C beträgt und die Anfangstemperatur, bei der der gewalzte Stahl auf das Kühlbett gelegt wird, 900-960 °C beträgt.

## Revendications

1. Barre d'armature en acier, **caractérisée en ce qu'**elle comprend les ingrédients suivants calculés en pourcentage pondéral :
0,005%-0,030% de C,
0,3%-0,6% de Si,
1,2%-2,5% de Mn,
0,01% ou moins de P,
0,01% ou moins de S,
8,0%-10,0% de Cr,
1,0%-3,0% de Mo,
0,2%-0,4% de Sn,
0,01%-0,05% d'élément des terres rares,
0,04%-0,18% de V et/ou 0,010%-0,030% de Ti,
et le reste étant Fe et des impuretés inévitables.

2. Barre d'armature en acier selon la revendication 1, **caractérisée en ce qu'**elle comprend les ingrédients suivants calculés en pourcentage pondéral :
0,005%-0,030% de C,
0,3%-0,6% de Si,
1,7%-2,5% de Mn,
0,01% ou moins de P,
0,01% ou moins de S,
8,0%-10,0% de Cr,
1,5%-2,0% de Mo,
0,2%-0,4% de Sn,
0,01%-0,05% d'élément des terres rares,
0,04%-0,08% de V, et
le reste étant Fe et des impuretés inévitables.

3. Barre d'armature en acier selon la revendication 1, **caractérisée en ce qu'**elle comprend les ingrédients suivants calculés en pourcentage pondéral :
0,005%-0,030% de C,
0,3%-0,6% de Si,
1,7%-2,5% de Mn,
0,01% ou moins de P,
0,01% ou moins de S,
8,0%-10,0% de Cr,
1,8%-3,0% de Mo,
0,2%-0,4% de Sn,
0,01%-0,05% d'élément des terres rares,
0,10%-0,18% de V,
0,010%-0,030% de Ti, et
le reste étant Fe et des impuretés inévitables.

4. Barre d'armature en acier selon l'une quelconque des revendications 1-3, **caractérisée en ce que** la barre d'armature en acier a une structure microscopique composée de ferrite et de bainite, la ferrite représentant un pourcentage de 50%-70%.

5. Barre d'armature en acier selon l'une quelconque des revendications 1-4, **caractérisée en ce que**
la barre d'armature en acier a un rapport entre la résistance à la traction et la limite d'élasticité supérieur à 1,25, un pourcentage d'allongement total à la contrainte maximale supérieur à 9% et un pourcentage d'allongement après fracture supérieur à 18%, mesurés selon la norme GB1499.2-2007 ;
la barre d'armature en acier a un taux de corrosion par essai de corrosion par immersion cyclique inférieur à 0,45 m²h et un taux de corrosion par essai de corrosion au brouillard salin inférieur à 0,45 m²h, mesurés selon GBT10125-1997.

6. Procédé de production d'une barre d'armature en acier, **caractérisé en ce qu'**il comprend les étapes suivantes :
S1 : réaliser une désulfuration préliminaire du fer fondu pour maintenir la teneur en soufre inférieure ou égale à 0,01% ;
S2 : réaliser une fusion dans un convertisseur, en alimentant conjointement le fer fondu traité par l'étape S1 et des déchets d'acier et/ou de la fonte brute dans le convertisseur en vue de leur fusion, pour obtenir ainsi un acier doté d'une teneur en carbone inférieure à 0,05% et d'une teneur en phosphore inférieure à 0,01% pour la coulée en poche de l'acier ;
S3 : réaliser la coulée en poche de l'acier, processus pendant lequel des éléments d'alliage de Si et Mn sont ajoutés pour la désoxygénation et de la poudre de carbone et de l'agent de formation de scories sont également ajoutés ;
S4 : réaliser le raffinage à l'extérieur du convertisseur, en ajoutant du Cr élémentaire et réaliser, entre-temps, la décarburation par insufflation d'oxygène dans un four de raffinage sous vide RH (Ruhrstahl Heraeur) de sorte à maintenir les teneurs en Cr et en C dans la plage selon l'une quelconque des revendications 1-3 ; effectuer la désoxygénation à l'aide d'un four LF (laddle furnace-four à poche de coulée), ajouter les éléments d'alliage requis de Mn, Mo, Sn, terres rares, ainsi que V et/ou Ti, dans l'acier après désoxygénation et ajouter ensuite l'alliage calcium-fer sous agitation douce par insufflation de gaz inerte, de sorte à maintenir les teneurs en ces éléments dans la plage selon l'une quelconque des revendications 1-3 ; élever la température de l'acier fondu et ajouter un agent de couverture ;
S5 : réaliser une coulée continue, en coulant l'acier fondu sous coulage protecteur à l'aide d'une machine de coulée pour former une brame de coulée continue.
S6 : réaliser le laminage, en chauffant la brame de coulée continue à une température supérieure à sa température d'austénitisation dans un four de chauffage, en effectuant un laminage brut, un laminage modéré, un laminage de précision, et placer l'acier laminé après le laminage de précision sur lit de refroidissement pour le refroidissement par air, pour produire un produit fini de type barre d'armature en acier doté des ingrédients selon l'une quelconque des revendications 1-3.

7. Procédé de production selon la revendication 6, **caractérisé en ce que**, dans l'étape S2, l'acier pour la coulée en poche de l'acier a une température inférieure ou égale à 1690°C.

8. Procédé de production selon la revendication 6 ou 7, **caractérisé en ce que**, dans l'étape S3, un gaz protecteur est insufflé dans l'acier fondu pour l'agitation pendant le processus de coulée en poche de l'acier.

9. Procédé de production selon l'une quelconque des revendications 6-8, **caractérisé en ce que** dans l'étape S4, la décarburation par insufflation d'oxygène est réalisée à une température supérieure ou égale à 1605°C pendant le raffinage dans le four de raffinage sous vide RH, la désoxygénation est réalisée à une température supérieure ou égale à 1575°C pendant le raffinage dans le four LF, pour maintenir la teneur en oxygène à au plus 50 ppm, l'agitation douce est réalisée pendant une durée supérieure ou égale à 5 min et la température de l'acier fondu est élevée à 1570-1600°C.

10. Procédé de production selon l'une quelconque des revendications 6-9, **caractérisé en ce que** dans l'étape S6, la brame de coulée continue est chauffée à 1100-1200°C dans le four de chauffage, la température de départ du laminage, avant le laminage brut, est de 1030-1100°C, la température pendant le laminage de précision est de 950-1050°C et la température lorsque l'acier laminé est initialement placé sur le lit de refroidissement est de 900-960°C.
